

## UNITED STATES PATENT OFFICE

2,095,220

## CUPRAMMONIUM YARN MANUFACTURE

August Hartmann, Berlin-Lichterfelde, Germany, assignor to American Bemberg Corporation, New York, N. Y., a corporation of Delaware

No Drawing. Application November 15, 1933, Serial No. 698,146. In Germany April 15, 1933

## 5 Claims. (Cl. 18—54)

Until the present time, the principal requirement for the production of commercial artificial silk from copper cellulose solutions, has been the use of softened water, provided such solutions are being spun in funnels under normal spinning conditions. Experiments have shown that by using hard instead of soft water under normal spinning conditions, i. e., with hole diameters of 0.8 to 1.0 mm., speeds of more than 25 meters per minute 5 and coagulating bath temperatures above 35° C., a product of inferior quality is obtained, and it is impossible to produce a continuous thread in this manner. It has been ascertained that these deficiencies are caused by too rapid a coagulation 10 of the spinning solution which is brought about by the salts contained in natural well water. The strong coagulating effect is mainly due to calcium carbonate present which forms the principal ingredient of the salts dissolved in such water, and, thus, it becomes practically impossible to obtain, 15 with well water of about 4 German degrees of total hardness, under normal spinning conditions, marketable products. The other constituents of such hard water, for example, calcium chloride or calcium sulfate, act to a lesser extent in an 20 analogous manner.

One object of my present invention is the use 25 of hard water containing especially calcium bicarbonate. I have found by experimentation that the use of calcium bicarbonate containing water is possible provided the wide openings of 0.8 mm. in diameter and above, heretofore employed, are replaced by nozzle openings the diameters of which have been considerably reduced, and do not exceed 0.6 mm. The temperatures of the coagulating bath may, as usual, be kept within a 30 range of from 30 to 40° C. It is to be noted, however, that lower temperatures, as low as 20° C., may be used. Since, especially, the calcium bicarbonate exerts a strong precipitating action, 35 the spinning conditions must be adjusted according to the calcium bicarbonate content of the water. In order to obtain the best results, the following rule has been found and must be strictly adhered to:

"The higher the bicarbonate content of water present, i. e., the so-called transient hardness, the smaller should be the diameter of the nozzle openings."

40 In other words the hole diameter must be reduced as a direct function of the water hardness. When extremely hard water, for example, of more than 10 German degrees of hardness, is used, it is advisable to operate with nozzle openings 45 having diameters smaller than 0.6 mm. and pref-

erably with openings of about 0.2 mm. in diameter.

The effect of the novel process which is characterized by the combined use of hard water and relatively narrow nozzle openings, is depicted in the following table:

## Normal copper cellulose solution

| Hole diameter | Hardness of water | Temperature | Spinning mass per min. | Spinning speed per min. | Resulting thread                                                          | 10 |
|---------------|-------------------|-------------|------------------------|-------------------------|---------------------------------------------------------------------------|----|
| 0.8 mm....    | 11° (German)      | ° C. 30     | cc. 700                | Meters 30               | Breaks in funnel spinning. impossible.                                    | 15 |
| 0.2 mm....    | 11° (German)      | 30          | 700                    | 30                      | Thread does not break inside or outside the funnel. Undisturbed spinning. | 20 |

This table clearly shows that continuous threads can be produced by spinning copper cellulose solutions into hard water provided the hole diameters of the spinning nozzles are reduced, and that threads extruded into hard water through openings of normal size will not allow the manufacture of a marketable product.

The following are two examples of spinning conditions which may be employed according to the invention, it being understood that these are given only by way of illustration and that the spinning conditions can be varied without departing from the spirit and scope of the present invention.

## Example 1

|                               |                                      |
|-------------------------------|--------------------------------------|
| Titer.....                    | 120 deniers                          |
| Single filament.....          | 1.3 deniers                          |
| Speed.....                    | 30 meters per minute                 |
| Water.....                    | 700 cc. of hard water (hardness 11°) |
| Temperature of water.....     | 25° C.                               |
| Hole diameter of nozzles..... | 0.15 millimeter                      |

## Example 2

|                               |                                  |
|-------------------------------|----------------------------------|
| Titer.....                    | 120 deniers                      |
| Single filament.....          | 1.3 deniers                      |
| Speed.....                    | 30 meters per minute             |
| Water.....                    | Containing 0.1% calcium chloride |
| Temperature of water.....     | 35° C.                           |
| Hole diameter of nozzles..... | 0.2 millimeter                   |

I claim:

1. In the stretch-spinning process of producing

5

25

30

35

40

45

50

55

- artificial silk, the step comprising extruding a cuprammonium cellulose solution through a nozzle opening of about 0.15 to 0.6 millimeter in diameter into water, the said water having a hardness of more than 10 German degrees and a temperature of about 20 to 35° C., the diameter of the nozzle opening being reduced within the range 0.15 to 0.6 millimeter as the hardness of the water increases.
2. In the stretch-spinning process of producing cuprammonium cellulose filaments of about 1.3 deniers, the step comprising extruding a cuprammonium cellulose solution at a speed of about 30 meters per minute through a nozzle opening of about 0.15 millimeter in diameter into water, said water having a hardness of about 11 German degrees and a temperature of about 25° C.
3. In the stretch-spinning process of producing cuprammonium cellulose filaments, the step comprising extruding a cuprammonium cellulose solution at a speed of about 30 meters per minute through a nozzle opening of about 0.2 milli-
- meters in diameter into water, said water having a hardness of about 11 German degrees and a temperature of about 30° C.
4. In the stretch-spinning process of producing artificial silk, the step comprising extruding a cuprammonium solution through a nozzle having openings of a diameter of about 0.15 to 0.6 millimeter into very hard water, the said water having a hardness of above 10 German degrees, the diameter of the said nozzle opening varying within the range of 0.15 to 0.6 in inverse ratio to the increasing hardness of the water above 10 German degrees.
5. In the stretch-spinning process of producing artificial silk by forcing a cuprammonium cellulose solution through suitable openings into hard water having a hardness of over 4 German degrees, the method comprising determining the hardness of the said water and selecting diameters of 0.6 millimeter to 0.15 millimeter as an inverse function of the hardness of the water.

AUGUST HARTMANN.